



US005662746A

**United States Patent** [19]**Affinito**[11] **Patent Number:** **5,662,746**[45] **Date of Patent:** **Sep. 2, 1997**

[54] **COMPOSITION AND METHOD FOR  
TREATMENT OF PHOSPHATED METAL  
SURFACES**

[75] Inventor: **John C. Affinito**, McHenry, Ill.

[73] Assignee: **Brent America, Inc.**, La Mirada, Calif.

[21] Appl. No.: **605,959**

[22] Filed: **Feb. 23, 1996**

[51] **Int. Cl.<sup>6</sup>** ..... **C23C 22/83**

[52] **U.S. Cl.** ..... **148/247; 148/257**

[58] **Field of Search** ..... **148/257, 247**

[56] **References Cited**

U.S. PATENT DOCUMENTS

3,684,587 8/1972 Geering ..... 148/257  
3,695,942 10/1972 Binns .....  
3,697,331 10/1972 Shatz ..... 148/257  
3,749,611 7/1973 Leon ..... 148/257

3,912,548 10/1975 Faigen ..... 148/247  
3,961,992 6/1976 Jahncke ..... 148/257  
4,457,790 7/1984 Lindert et al. ....  
4,517,028 5/1985 Lindert .....  
4,650,526 3/1987 Claffey et al. ....  
4,656,097 4/1987 Claffey et al. ....  
5,246,507 9/1993 Kodama ..... 148/257

*Primary Examiner*—Sam Silverberg

*Attorney, Agent, or Firm*—Pretty, Schroeder & Poplawski

[57] **ABSTRACT**

A rinse solution for the treatment of conversion-coated metal substrates for improving the adhesion and corrosion resistance of siccative coatings, comprising an aqueous solution of a Group IVA metal ion, namely, zirconium, titanium, hafnium, and mixtures thereof, and a phenol polymer, with the pH of the total solution about 3.5 to 5.1. A method for treating such materials by applying the rinse solution to the substrate.

**37 Claims, No Drawings**

**COMPOSITION AND METHOD FOR  
TREATMENT OF PHOSPHATED METAL  
SURFACES**

**BACKGROUND OF THE INVENTION**

This invention relates to the treatment of metal surfaces prior to a finishing operation, such as the application of a siccative organic coating (also known as an "organic coating", "organic finish", or simply, "paint"). Specifically, this invention relates to the treatment of conversion-coated metal with an aqueous solution comprising a phenolic resin and a Group IVA metal ion, namely zirconium, titanium, hafnium, and mixtures thereof. Treatment of conversion-coated metal with such a solution improves paint adhesion and corrosion resistance.

The primary purposes of applying siccative coatings to metal substrates (e.g., steel, aluminum, zinc and their alloys) are protection of the metal surface from corrosion and for aesthetic reasons. It is well-known, however, that many organic coatings adhere poorly to metals in their normal state. As a result, corrosion-resistance characteristics of the siccative coating are substantially diminished. It is therefore a typical procedure in the metal finishing industry to subject metals to a pretreatment process whereby a conversion coating is formed on the metal surface. This conversion coating acts as a protective layer, slowing the onset of the degradation of the base metal, owing to the conversion coating being less soluble in a corrosive environment than is the base metal. The conversion coating is also effective by serving as a recipient for a subsequent siccative coating. The conversion coating has a greater surface area than does the base metal and thus provides for a greater number of adhesion sites for the interaction between the conversion coating and the organic finish. Typical examples of such conversion coatings include, but are not limited to, iron phosphate coatings, zinc phosphate coatings, and chromate conversion coatings. These conversion coatings and others are well-known in the art and will not be described in any further detail.

Normally, the application of an organic finish to a conversion-coated metal surface is not sufficient to provide the highest levels of paint adhesion and corrosion resistance. Painted metal surfaces are able to reach maximum performance levels when the conversion-coated metal surface is treated with a "final rinse", also referred to in the art as a "post-rinse" or a "seal rinse", prior to the painting operation. Final rinses are typically aqueous solutions containing organic or inorganic entities designed to improve paint adhesion and corrosion resistance. The purpose of any final rinse, regardless of its composition, is to form a system with the conversion coating in order to maximize paint adhesion and corrosion resistance. This may be accomplished by altering the electrochemical state of the conversion-coated substrate by rendering it more passive or it may be accomplished by forming a barrier film which prevents a corrosive medium from reaching the metal surface. The most effective final rinses in general use today are aqueous solutions containing chromic acid, partially reduced to render a solution comprising a combination of hexavalent and trivalent chromium. Final rinses of this type have long been known to provide the highest levels of paint adhesion and corrosion resistance. Chromium-containing final rinses, however, have a serious drawback due to their inherent toxicity and their hazardous nature. These concerns make chromium-containing final rinses less desirable from a practical standpoint, when one considers such issues as safe handling of chemicals and the environmental problems associated with the discharge of such solutions into municipal water streams. Thus, it has been a goal of the industry to find

chromium-free alternatives which are less toxic and more environmentally benign than chromium-containing final rinses. It has also been desirous to develop chromium-free final rinses which are as effective as chromium-containing final rinses in terms of paint adhesion and corrosion resistance properties.

Much work has already been done in the area of chromium-free final rinses. Some of these have utilized either Group IVA chemistry or phenolic polymers. U.S. Pat. No. 3,695,942 describes a method of treating conversion-coated metal with an aqueous solution containing soluble zirconium compounds. U.S. Pat. No. 4,650,526 describes a method of treating phosphated metal surfaces with an aqueous mixture of an aluminum zirconium complex, an organofunctional ligand and a zirconium oxyhalide. The treated metal could be optionally rinsed with deionized water prior to painting. U.S. Pat. No. 4,457,790 describes a treatment composition utilizing titanium, zirconium and hafnium in aqueous solutions containing polymers with chain length from 1 to 5 carbon atoms. U.S. Pat. No. 4,656,097 describes a method for treating phosphated metal surfaces with organic titanium chelates. The treated metal surface can optionally be rinsed with water prior to the application of a siccative organic coating. U.S. Pat. No. 4,497,656 details a process for treating phosphated metal surfaces with solutions containing trivalent titanium and having a pH of 2 to 7. U.S. Pat. No. 4,457,790 and U.S. Pat. No. 4,517,028 describe a final rinse composition comprising a polyalkylphenol and Group IVA metal ion. In all of the above examples, the treatment method described claimed to improve paint adhesion and corrosion resistance.

The levels of paint adhesion and corrosion resistance afforded by the treatment solutions in the above examples do not reach the levels desired by the metal finishing industry, namely the performance characteristics of chromium-containing final rinses. I have found that aqueous solutions containing a phenolic resin and Group IVA metal ions, namely, zirconium, titanium, hafnium, and mixtures thereof, provide paint adhesion and corrosion resistance characteristics comparable to those attained with chromium-containing final rinses. In many cases, the performance of conversion-coated metal surfaces treated with phenolic resin-Group IVA metal ion solutions in accelerated corrosion tests exceeds that of conversion-coated metal treated with chromium-containing solutions.

**SUMMARY OF THE INVENTION**

It is an object of this invention to provide a method and composition of an aqueous rinse which will impart an improved level of paint adhesion and corrosion resistance on painted, conversion-coated metal. The composition comprises an aqueous solution containing a phenolic resin and a Group IVA metal ion, namely, zirconium, titanium, hafnium, and mixtures thereof, and provides levels of paint adhesion and corrosion resistance comparable to or exceeding those provided by chromium-containing final rinses.

It is a further object of the invention to provide a method and rinse composition which contains no chromium.

The presently preferred embodiment of the invention includes a rinse solution for the treatment of conversion-coated metal substrates for improving the adhesion and corrosion resistance of siccative coatings, comprising an aqueous solution of a Group IVA metal ion, namely, zirconium, titanium, hafnium, and mixtures thereof, and a phenolic resin, with the solution having a pH of about 3.5 to 5.1.

The invention also includes a method for treating such materials by applying the rinse solution to the substrate.

**DESCRIPTION OF THE PREFERRED  
EMBODIMENTS**

The rinse solution of the invention is an aqueous solution containing a phenolic resin and Group IVA metal ion,

namely, zirconium, titanium, hafnium, and mixtures thereof. It is intended that the rinse solution be applied to conversion-coated metal. The formation of conversion coatings on metal substrates is well-known within the metal finishing industry. In general, this process is usually described as a process requiring several pretreatment stages. The actual number of stages is typically dependent on the final use of the painted metal article. The number of pretreatment steps normally varies anywhere from two to nine stages. A representative example of a pretreatment process involves a five-stage operation where the metal which will ultimately be painted goes through a cleaning stage, a water rinse, a conversion coating stage, a water rinse and a final rinse stage. Modifications to the pretreatment process can be made according to specific needs. As an example, surfactants can be incorporated into some conversion coating baths so that cleaning and the formation of the conversion coating can be achieved simultaneously. In other cases it may be necessary to increase the number of pretreatment stages so as to accommodate more pretreatment steps. Examples of the types of conversion coatings that can be formed on metal substrates are iron phosphates and zinc phosphates. Iron phosphating is usually accomplished in no more than five pretreatment stages, while zinc phosphating usually requires a minimum of six pretreatment stages. The number of rinse stages between the actual pretreatment steps can be adjusted to ensure that rinsing is complete and effective and so that the chemical pretreatment from one stage is not carried on the metal surface to subsequent stages, thereby possibly contaminating them. It is typical to increase the number of rinse stages when the metal parts to be treated have unusual geometries or areas that are difficult for the rinse water to contact. The method of application of the pretreatment operation can be either an immersion or a spray operation. In immersion operations, the metal articles are submerged in the various pretreatment baths for defined intervals before moving on to the next pretreatment stage. A spray operation is one where the pretreatment solutions and rinses are circulated by means of a pump through risers fashioned with spray nozzles. The metal articles to be treated normally proceed through the pretreatment operation by means of a continuous conveyor. Virtually all pretreatment processes can be modified to run in spray mode or immersion mode, and the choice is usually made based on the final requirements of the painted metal article. It is to be understood that the invention described here can be applied to any conversion-coated metal surface and can be applied either as a spray process or an immersion process.

The rinse solution of the invention comprises an aqueous solution of a phenolic resin and Group IVA metal ion. Specifically, the rinse solution is an aqueous solution containing zirconium, titanium, or hafnium ions, and mixtures thereof, whose source can be hexafluorozirconic acid, hexafluorotitanic acid, hafnium oxide, titanium oxysulfate, titanium tetrafluoride, zirconium sulfate and mixtures thereof, and a phenolic resin which is a phenol polymer with formaldehyde. The phenolic resin is a water soluble base catalyzed condensation product of the reaction between phenol and formaldehyde. A present source for such resin is Schenectady International, Inc. SP-6877. The resin is typically a mixture of substituted phenol compounds, namely: 2-hydroxybenzyl alcohol, 4-hydroxybenzyl alcohol, 2,6-dimethylol phenol, 2,4-dimethylol phenol and 2,4,6-trimethylol phenol.

The rinse solution is prepared by making an aqueous solution using deionized water. The solution contains: a Group IVA metal ion, namely, zirconium, titanium, hafnium, and mixtures thereof, such that the metal ion concentration is about 0.00035% w/w to about 0.005% w/w and that of the phenol polymer is about 0.01% w/w to about 0.4% w/w. The aqueous solution also contains a water-soluble solvent such

as tripropylene glycol monomethyl ether to make the solution homogeneous. The pH of the resulting solution is adjusted to about 3.5 to 5.1 using sodium hydroxide.

5 A preferred version of the invention is an aqueous solution containing 0.00035 to 0.0016% w/w titanium ion and 0.01 to 0.40% w/w of phenol polymer. The resulting solution can be effectively operated at pH 3.5 to 5.1.

10 Another preferred version of the invention is an aqueous solution containing 0.00065 to 0.0050% w/w zirconium ion and 0.01 to 0.40% w/w of phenol polymer. The resulting solution can be effectively operated at pH 3.5 to 5.1.

15 Another preferred version of the invention is an aqueous solution containing 0.00035 to 0.0050% w/w hafnium ion and 0.01 to 0.40% w/w of phenol polymer. The resulting solution can be effectively operated at pH 3.5 to 5.1.

20 An especially preferred version of the invention is an aqueous solution containing 0.00035 to 0.0010% w/w titanium ion and 0.01 to 0.077% w/w of phenol polymer. The resulting solution can be effectively operated at pH 4.0 to 5.1.

25 Another especially preferred version of the invention is an aqueous solution containing 0.00065 to 0.0011% w/w zirconium ion and 0.01 to 0.077% w/w of phenol polymer. The resulting solution can be effectively operated at pH 4.0 to 5.1.

30 Another especially preferred version of the invention is an aqueous solution containing 0.0008 to 0.0010% w/w hafnium ion and 0.01 to 0.077% w/w of phenol polymer. The resulting solution can be effectively operated at pH 4.0 to 5.1.

35 The rinse solution of the invention can be applied by various means, so long as contact between the rinse solution and the conversion-coated substrate is effected. The preferred methods of application of the rinse solution of the invention are by immersion or by spray. In an immersion operation, the conversion-coated metal article is submerged in the rinse solution of the invention for a time interval from about 5 sec to 5 min, preferably 45 sec to 1 min. In a spray operation, the conversion-coated metal article comes in contact with the rinse solution of the invention by means of

40 pumping the rinse solution through risers fashioned with spray nozzles. The application interval for the spray operation is about 5 sec to 5 min, preferably 45 sec to 1 min. The rinse solution of the invention can be applied at temperatures from about 70° F. to 150° F., preferably 70° F. to 90° F.

45 Following treatment in the rinse solution, the treated metal article can be optionally post-rinsed with deionized water. The use of such a post-rinse is common in many industrial electrocoating operations. The conversion-coated metal article treated with the rinse solution of the invention can be dried by various means, preferably oven drying at about 350° F. for about 5 min. The conversion-coated metal article, now treated with the rinse solution of the invention, is ready for application of the siccative coating.

## EXAMPLES

55 The following examples demonstrate the utility of the rinse solution of the invention. Comparative examples include conversion-coated metal substrates treated with a chromium-containing rinse and conversion-coated metal substrates treated with a final rinse solution as described in U.S. Pat. No. 4,517,028, which is a final rinse composition comprising a polyalkylphenol and Group IVA metal ion. Another comparative example was to treat conversion-coated metal substrates with a deionized-water final rinse. Throughout the examples, specific parameters for the pre-treatment process, for the rinse solution of the invention, for the comparative rinses and the nature of the substrate and the type of siccative coating are described.

60 65

Some of the panels described in the various examples were painted with three different electrocoatings, all applied anodically. These were: Vectrocoat 300 Gray and Vectrocoat 300 Red, both acrylics, and both manufactured by the Valspar Corporation, Garland, Tex. The third electrocoat was Unichem E-2000, manufactured by Universal Chemicals & Coatings, Elgin Ill. Two other organic coatings that were applied to some of the panels were a melamine-modified polyester and a water-based coating, both manufactured by the Sheboygan Paint Company, Sheboygan, Wis.

All treated and painted metal samples were subjected to accelerated corrosion testing. In general, the testing was performed according to the guidelines specified in ASTM B-117-90. Specifically, three identical specimens were prepared for each pretreatment system. The painted metal samples received a single, diagonal scribe which broke through the organic finish and penetrated to bare metal. All unpainted edges were covered with electrical tape. The specimens remained in the salt spray cabinet for an interval that was commensurate with the type of siccative coating that was being tested. Once removed from the salt spray cabinet, the metal samples were rinsed with tap water, dried by blotting with paper towels and evaluated. The evaluation was performed by scraping away the loose paint and corrosion products from the scribe area with the flat end of a spatula. The scraping was performed in such a manner so as only to remove loose paint and leave adhering paint intact. In the case of some organic finishes, removal of the loose paint and corrosion products from the scribe was accomplished by means of a tape pull as specified in ASTM B-117-90. Once the loose paint was removed, the scribe areas on the specimens were then measured to determine the amount of paint lost due to corrosion creepage. Each scribe line was measured at eight intervals, approximately 1 mm apart, measured across the entire width of the scribe area. The eight values were averaged for each specimen and the averages of the three identical specimens were averaged to arrive at the final result. The creepage values reported in the following tables reflect these final results.

#### Example 1

Cold-rolled steel test panels from Advanced Coating Technologies, Hillsdale, Mich. were processed through a five-stage pretreatment operation. The panels were cleaned with Brent America, Inc. Chem Clean 1303, a commercially available alkaline cleaning compound. Once rendered water-break-free, the test panels were rinsed in tap water and phosphated with Brent America, Inc. Chem Cote 3011, a commercially available iron phosphate. The phosphating bath was operated at about 6.2 points, 140° F., 3 min contact time, pH 4.8. After phosphating, the panels were rinsed in tap water and treated with various final rinse solutions for 1 min. The panels were given a deionized-water post-rinse prior to dry-off. The comparative chromium-containing rinse was Brent America, Inc. Chem Seal 3603, a commercially available product. This bath was run at 0.25% w/w. In accordance with normal practice in the metal finishing industry, panels treated with the chromium-containing final rinse (1) were rinsed with deionized water prior to dry-off. Panels treated with the comparative chromium-free final rinse (2) were obtained from Advanced Coating Technologies, Hillsdale, Mich. identified by Code APR20809. All panels treated in the laboratory were then dried in an oven at 350° F. for 5 min. The panels were painted with Vectrocoat 300 Gray, Vectrocoat 300 Red, Unichem E-2000, the water-based coating, and the melamine-modified polyester. The various rinses studied are summarized as follows.

1. Chem Seal 3603, chromium-containing final rinse.
2. Comparative chromium-free final rinse.

3. Phenol polymer, 0.01% w/w, pH 4.00, Ti concentration, 0.00035% w/w.
4. Phenol polymer, 0.50% w/w, pH 4.00, Ti concentration, 0.00035% w/w.
5. Phenol polymer, 0.30% w/w, pH 4.00, Ti concentration, 0.00035% w/w.
6. Phenol polymer, 0.40% w/w, pH 4.00, Ti concentration, 0.00035% w/w.

The salt spray results are described in Tables I and II and III. The values represent total creepage about the scribe area in mm. The numbers in parentheses represent the exposure interval for that particular organic finish.

#### Example 2

- 15 Another set of cold-rolled steel test panels was prepared using the parameters described in Example 1. The conversion-coated test panels were painted with Vectrocoat 300 Gray, Vectrocoat 300 Red, and the water-based coating. The various final rinses are summarized as follows.
- 20 1. Chem Seal 3603, chromium-containing final rinse.
  2. Comparative chromium-free final rinse.
  7. Phenol polymer, 0.077% w/w, pH 4.00, Ti concentration, 0.00035% w/w.
  8. Phenol polymer, 0.077% w/w, pH 4.00, Ti concentration, 0.00060% w/w.
  - 25 9. Phenol polymer, 0.077% w/w, pH 4.00, Ti concentration, 0.00085% w/w.
  10. Phenol polymer, 0.077% w/w, pH 4.00, Ti concentration, 0.00110% w/w.
  11. Phenol polymer, 0.077% w/w, pH 4.00, Ti concentration, 0.00135% w/w.
  12. Phenol polymer, 0.077% w/w, pH 4.00, Ti concentration, 0.00160% w/w.
  13. Phenol polymer, 0.077% w/w, pH 4.00, Ti concentration, 0.00185% w/w.

The salt spray results are described in Table IV. The values represent total creepage about the scribe area in mm. The numbers in parentheses represent the exposure interval for that particular organic finish.

#### Example 3

- Another set of cold-rolled steel test panels was prepared using the parameters described in Example 1. The conversion-coated test panels were painted with Vectrocoat 300 Gray, Vectrocoat 300 Red, Unichem E-2000, and the melamine-modified polyester. The various final rinses are summarized as follows.
1. Chem Seal 3603, chromium-containing final rinse.
  2. Comparative chromium-free final rinse.
  - 50 14. Phenol polymer, 0.077% w/w, pH 3.50, Ti concentration, 0.00035% w/w.
  15. Phenol polymer, 0.077% w/w, pH 5.10, Ti concentration, 0.00035% w/w.
  16. Phenol polymer, 0.077% w/w, pH 3.00, Ti concentration, 0.00035% w/w.
  - 55 17. Phenol polymer, 0.077% w/w, pH 5.40, Ti concentration, 0.00035% w/w.
- The salt spray results are described in Tables V and VI. The values represent total creepage about the scribe area in mm. The numbers in parentheses represent the exposure interval for that particular organic finish.

#### Example 4

- Another set of cold-rolled steel test panels was prepared using the parameters described in Example 1. The final rinse was applied by an immersion technique on some conversion-coated panels and was applied by means of a

recirculating spray on others. The conversion-coated test panels were painted with Vectrocoat 300 Gray, Vectrocoat 300 Red, Unichem E-2000, and the melamine-modified polyester. The various final rinses are summarized as follows.

7. Phenol polymer, 0.077% w/w, pH 4.00, Ti concentration, 0.00035% w/w, spray application.
18. Phenol polymer, 0.077% w/w, pH 4.00, Ti concentration, 0.00035% w/w, immersion application.

The salt spray results are described in Table VII. The values represent total creepage about the scribe area in mm. The numbers in parentheses represent the exposure interval for that particular organic finish.

#### Example 5

Another set of cold-rolled steel test panels was prepared using the parameters described in Example 1. The conversion-coated test panels were painted with Vectrocoat 300 Red and the water-based coating. The various final rinses are summarized as follows.

1. Chem Seal 3603, chromium-containing final rinse.
19. Phenol polymer, 0.077% w/w, pH 4.00, Ti concentration, 0.00035% w/w, Zr concentration, 0.00066% w/w.
20. Phenol polymer, 0.077% w/w, pH 4.00, Ti concentration, 0.00035% w/w, Hf concentration, 0.00035% w/w.
21. Phenol polymer, 0.077% w/w, pH 4.00, Zr concentration, 0.00066% w/w, Hf concentration, 0.00035% w/w.
22. Phenol polymer, 0.077% w/w, pH 4.00, Ti concentration, 0.00035% w/w, Zr concentration, 0.00066% w/w, Hf concentration, 0.00035% w/w.

The salt spray results are described in Table VIII. The values represent total creepage about the scribe area in mm. The numbers in parentheses represent the exposure interval for that particular organic finish.

#### Example 6

Another set of cold-rolled steel test panels was prepared using the parameters described in Example 1. The conversion-coated test panels were painted with Vectrocoat 300 Red, Vectrocoat Gray, Unichem E-2000, the melamine-modified polyester and the water-based coating. The various final rinses are summarized as follows.

1. Chem Seal 3603, chromium-containing final rinse.
23. Phenol polymer, 0.077% w/w, pH 4.00, Zr concentration, 0.00065% w/w.
24. Phenol polymer, 0.077% w/w, pH 4.00, Zr concentration, 0.0050% w/w.
25. Phenol polymer, 0.077% w/w, pH 4.00, Zr concentration, 0.0011% w/w.
26. Phenol polymer, 0.077% w/w, pH 4.00, Hf concentration, 0.0010% w/w.
27. Phenol polymer, 0.077% w/w, pH 4.00, Hf concentration, 0.0008% w/w.
28. Phenol polymer, 0.077% w/w, pH 4.00, Hf concentration, 0.0050% w/w.

The salt spray results are described in Tables IX, X, XI and XII. The values represent total creepage about the scribe

area in mm. The numbers in parentheses represent the exposure interval for that particular organic finish.

#### Example 7

Another set of cold-rolled steel test panels was prepared using the parameters described in Example 1. The conversion-coated test panels were painted with Vectrocoat 300 Red and Vectrocoat 300 Gray. The various final rinses are summarized as follows.

1. Chem Seal 3603, chromium-containing final rinse.
29. Phenol polymer, 0.077% w/w, pH 4.00, Ti concentration, 0.00035% w/w.
30. Phenol polymer, 0.077% w/w, pH 4.00, Zr concentration, 0.00065% w/w.

The salt spray results are described in Table XIII. The values represent total creepage about the scribe area in mm. The numbers in parentheses represent the exposure interval for that particular organic finish.

#### Example 8

Another set of cold-rolled steel test panels was prepared using the parameters described in Example 1. The conversion-coated test panels were painted with the melamine-modified polyester. The various final rinses are summarized as follows.

1. Chem Seal 3603, chromium-containing final rinse.
31. Phenol polymer, 0.077% w/w, pH 4.00, Ti concentration, 0.00035% w/w, followed by a deionized water post-rinse.
32. Phenol polymer, 0.077% w/w, pH 4.00, Ti concentration, 0.00035% w/w, without a deionized water post-rinse.

The salt spray results are described in Table XIV. The values represent total creepage about the scribe area in mm. The numbers in parentheses represent the exposure interval for that particular organic finish.

The results from accelerated corrosion testing demonstrated in Examples 1 to 8 show that rinse solutions containing a phenolic resin and a Group IVA metal ion provided substantially better performance than the comparative 40 chromium-free rinse, Rinse No. 2. The results demonstrated in Examples 1 to 8 also show that rinse solutions containing a phenolic resin and Group IVA metal ion, namely zirconium, titanium, hafnium and mixtures thereof, provided, in many cases, corrosion resistance comparable to that of a chromium-containing rinse, such as Final Rinse No. 1. In several instances, rinse solutions containing a phenolic resin and Group IVA metal ion, namely, zirconium, titanium, hafnium, and mixtures thereof, provided significantly higher levels of corrosion resistance than that achieved with a chromium-containing rinse.

The terms and expressions which have been employed are used as terms of description and not of limitation, and there is no intention in the use of such terms and expressions of excluding any equivalents of the features shown and described, or portions thereof, but it is recognized that various modifications are possible within the scope of the invention claimed.

TABLE I

| Final Rinse No. | 300 Gray (120 hr) | 300 Red (96 hr) | Unichem (504 hr) | Melamine (144 hr) |
|-----------------|-------------------|-----------------|------------------|-------------------|
| 1               | 7.8               | 9               | 7.3              | 8.3               |
| 2               | 10.5              | 14.7            | 4.2              | 8.8               |
| 3               | 7.9               | 9.4             | 4.3              | 14.8              |

TABLE II

| Final Rinse No. | 300 Gray (120 hr) | 300 Red (96 hr) | Unichem (504 hr) | Melamine (144 hr) |
|-----------------|-------------------|-----------------|------------------|-------------------|
| 1               | 15.5              | 11.2            | 14.3             | 6.1               |
| 4               | 16.8              | 21.9            | 14.9             | 32.7              |

TABLE III

| Final Rinse No. | 300 Gray (120 hr) | 300 Red (120 hr) | Water-based (168 hr) |
|-----------------|-------------------|------------------|----------------------|
| 1               | 14.7              | 16               | 7                    |
| 5               | 19.1              | 17               | 6.3                  |
| 6               | 10.4              | 10.2             | 6.1                  |

TABLE IV

| Final Rinse No. | 300 Gray (120 hr) | 300 Red (120 hr) | Water-based (168 hr) |
|-----------------|-------------------|------------------|----------------------|
| 1               | 12.1              | 11.5             | 5.7                  |
| 7               | 8.4               | 12.4             | 2.2                  |
| 8               | 3.5               | 6.7              | 2                    |
| 9               | 5.5               | 6.4              | 1.9                  |
| 10              | 5.8               | 7.5              | 2.4                  |
| 11              | 6.6               | 9.9              | 3                    |
| 12              | 9.2               | 11               | 3.3                  |
| 13              | 9.5               | 12.9             | 22.9                 |

TABLE V

| Final Rinse No. | 300 Gray (120 hr) | 300 Red (96 hr) | Unichem (504 hr) | Melamine (144 hr) |
|-----------------|-------------------|-----------------|------------------|-------------------|
| 1               | 7.8               | 9               | 7.3              | 8.3               |
| 2               | 10.5              | 14.7            | 4.2              | 8.8               |
| 14              | 8.8               | 9.5             | 5.1              | 10.3              |
| 15              | 6.2               | 5.8             | 6.5              | 3.9               |

TABLE VI

| Final Rinse No. | 300 Gray (120 hr) | 300 Red (96 hr) | Unichem (504 hr) | Melamine (144 hr) |
|-----------------|-------------------|-----------------|------------------|-------------------|
| 1               | 15.5              | 11.2            | 14.3             | 6.1               |
| 16              | 23.2              | 13.8            | 10.6             | 16.4              |
| 17              | 18.1              | 29.4            | 18.1             | 41.8              |

TABLE VII

| Final Rinse No. | 300 Gray (120 hr) | 300 Red (96 hr) | Unichem (504 hr) | Melamine (144 hr) |
|-----------------|-------------------|-----------------|------------------|-------------------|
| 7               | 4.3               | 4.7             | 4.7              | 4.5               |
| 18              | 7.1               | 3.3             | 9.4              | 3.5               |

TABLE VIII

| Final Rinse No. | Water-based (216 hr) | 300 Red (120 hr) |
|-----------------|----------------------|------------------|
| 1               | 4.1                  | 7.2              |
| 19              | 3.5                  | 6.2              |
| 20              | 2.7                  | 6.3              |

TABLE VIII-continued

| Final Rinse No. | Water-based (216 hr) | 300 Red (120 hr) |
|-----------------|----------------------|------------------|
| 21              | 2.6                  | 3.9              |
| 22              | 3.6                  | 6.6              |

TABLE IX

| Final Rinse No. | 300 Gray (120 hr) | 300 Red (96 hr) | Unichem (504 hr) | Melamine (144 hr) |
|-----------------|-------------------|-----------------|------------------|-------------------|
| 1               | 7.8               | 9               | 7.3              | 8.3               |
| 23              | 5.5               | 4.7             | 5.9              | 4                 |

TABLE X

| Final Rinse No. | 300 Red (96 hr) | 300 Gray (120 hr) | Unichem (336 hr) | Melamine (144 hr) |
|-----------------|-----------------|-------------------|------------------|-------------------|
| 1               | 15.9            | 24                | 20.4             | 28.9              |
| 25              | 7.3             | 10.9              | 2.6              | 38.6              |
| 26              | 5.3             | 6.5               | 1.6              | 5.5               |

TABLE XI

| Final Rinse No. | 300 Gray (120 hr) | 300 Red (96 hr) | Melamine (144 hr) |
|-----------------|-------------------|-----------------|-------------------|
| 1               | 56.7              | 17.2            | 30.5              |
| 27              | 11.7              | 5.8             | 1.9               |

TABLE XII

| Final Rinse No. | 300 Gray (120 hr) | 300 Red (96 hr) | Water-based (120 hr) |
|-----------------|-------------------|-----------------|----------------------|
| 1               | 24.7              | 20.8            | 24.5                 |
| 24              | 22.1              | 19.8            | 10.8                 |
| 28              | 9.3               | 12.9            | 10.7                 |

TABLE XIII

| Final Rinse No. | 300 Gray (96 hr) | 300 Red (96 hr) |
|-----------------|------------------|-----------------|
| 1               | 9                | 9.6             |
| 29              | 5.1              | 8.3             |
| 30              | 9.2              | N/A             |

TABLE XIV

| Final Rinse No. | Melamine (168 hr) |
|-----------------|-------------------|
| 1               | 8.8               |
| 31              | 6.1               |
| 32              | 2.4               |

The rinses numbers 3 through 32 provided results at least as good as the results for the conventional chromium rinse number 1, and are considered acceptable examples of the present invention. Rinses with compositions outside the ranges of rinses 3-32 were also tested but provided unacceptable results.

I claim:

1. A rinse solution for the treatment of conversion-coated metal substrates for improving the adhesion and corrosion resistance of siccative coatings, comprising an aqueous solution of a Group IVA metal ion, selected from the group consisting of zirconium, titanium, hafnium, and mixtures thereof, and a phenolic resin in a concentration of about 0.01 to 0.40% w/w, with the Group IVA metal ion in a concentration of about 0.00035 to 0.0050% w/w, and the pH for the entire solution about 3.5 to 5.1, with the phenolic resin being a water soluble base catalyzed condensation product of the reaction between phenol and formaldehyde.

2. A rinse solution as defined in claim 1 wherein the titanium ion concentration in the rinse solution is about

0.00035 to 0.0016% w/w and the phenolic resin concentration is about 0.01 to 0.40% w/w.

3. A rinse solution as defined in claim 1 wherein the titanium ion concentration in the rinse solution is about 0.00035 to 0.0016% w/w and the phenolic resin concentration is about 0.01 to 0.40% w/w, with a pH of about 3.5 to 5.1.

4. A rinse solution as defined in claim 1 wherein the titanium ion concentration in the rinse solution is about 0.00035 to 0.0010% w/w and the phenolic resin concentration is about 0.01 to 0.077% w/w, with a pH of about 4.0 to 5.1.

5. A rinse solution as defined in claim 1 wherein the zirconium ion concentration in the rinse solution is about 0.00065 to 0.0050% w/w and the phenolic resin concentration is about 0.01 to 0.40% w/w.

6. A rinse solution as defined in claim 1 wherein the zirconium ion concentration in the rinse solution is about 0.00065 to 0.0050% w/w and the phenolic resin concentration is about 0.01 to 0.40% w/w, with a pH of about 3.5 to 5.1.

7. A rinse solution as defined in claim 1 wherein the zirconium ion concentration in the rinse solution is about 0.00065 to 0.0011% w/w and the phenolic resin concentration is about 0.01 to 0.077% w/w, with a pH of about 4.0 to 5.1.

8. A rinse solution as defined in claim 1 wherein the hafnium ion concentration in the rinse solution is about 0.00035 to 0.0050% w/w and the phenolic resin concentration is about 0.01 to 0.40% w/w.

9. A rinse solution as defined in claim 1 wherein the hafnium ion concentration in the rinse solution is about 0.00035 to 0.0050% w/w and the phenolic resin concentration is about 0.01 to 0.40% w/w, with a pH of about 3.5 to 5.1.

10. A rinse solution as defined in claim 1 wherein the hafnium ion concentration in the rinse solution is about

0.0008 to 0.0010% w/w and the phenolic resin concentration is about 0.01 to 0.077% w/w, with a pH of about 4.0 to 5.1.

11. A rinse solution as defined in claim 1 wherein the titanium ion concentration in the rinse solution is about 0.00035 to 0.0016% w/w and the zirconium concentration is about 0.00065 to 0.0011% w/w and the phenolic resin concentration is about 0.01 to 0.077% w/w, with a pH of about 4.0 to 5.1.

12. A rinse solution as defined in claim 1 wherein the titanium ion concentration in the rinse solution is about 0.00035 to 0.0016% w/w and the hafnium concentration is about 0.00035 to 0.0050% w/w and the phenolic resin concentration is about 0.01 to 0.077% w/w, with a pH of about 4.0 to 5.1.

13. A rinse solution as defined in claim 1 wherein the hafnium ion concentration in the rinse solution is about 0.00035 to 0.0050% w/w and the zirconium concentration is about 0.00065 to 0.0011% w/w and the phenolic resin concentration is about 0.01 to 0.077% w/w, with a pH of about 4.0 to 5.1.

14. A rinse solution as defined in claim 1 wherein the titanium ion concentration in the rinse solution is about 0.00035 to 0.0016% w/w and the zirconium concentration is about 0.00065 to 0.0011% w/w and the hafnium ion concentration is about 0.00035 to 0.0050% w/w and the phenolic resin concentration is about 0.01 to 0.077% w/w, with a pH of about 4.0 to 5.1.

15. A rinse solution as defined in claim 1 wherein the titanium ion concentration in the rinse solution is about 0.00035 to 0.0010% w/w and the phenolic resin concentration is about 0.01 to 0.077% w/w, with a pH of about 4.0 to 5.1, where the solution is applied by means of spraying.

16. A rinse solution as defined in claim 1 wherein the titanium ion concentration in the rinse solution is about 0.00035 to 0.0010% w/w and the phenolic resin concentration is about 0.01 to 0.077% w/w, with a pH of about 4.0 to 5.1, where the solution is applied by means of dipping.

17. A rinse solution as defined in claim 1 wherein the Group IVA metal ion is from a Group IVA metal ion source selected from the group consisting of hexafluorozirconic acid, hexafluorotitanic acid, hafnium oxide, titanium oxysulfate, titanium tetrafluoride, zirconium sulfate and mixtures thereof.

18. In a method for treating conversion-coated metal substrates for improving the adhesion and corrosion resistance of siccative coatings, wherein the improvement comprises:

providing an aqueous solution of a Group IVA metal ion, selected from the group consisting of zirconium, titanium, hafnium, and mixtures thereof, and a phenolic resin in a concentration of about 0.01 to 0.40% w/w, with the phenolic resin being a water soluble base catalyzed condensation product of the reaction between phenol and formaldehyde;

providing the Group IVA metal ion concentration at about 0.00035 to 0.0050% w/w;

providing a pH of the solution of about 3.5 to 5.1; and applying the solution to the substrate.

19. The method as defined in claim 18 wherein the titanium ion concentration in the rinse solution is about 0.00035 to 0.0016% w/w and the phenolic resin concentration is about 0.01 to 0.40% w/w.

20. The method as defined in claim 18 wherein the titanium ion concentration in the rinse solution is about 0.00035 to 0.0016% w/w and the phenolic resin concentration is about 0.01 to 0.40% w/w, with a pH of about 3.5 to 5.1.

21. The method as defined in claim 18 wherein the titanium ion concentration in the rinse solution is about 0.00035 to 0.0010% w/w and the phenolic resin concentration is about 0.01 to 0.077% w/w, with a pH of about 4.0 to 5.1.

22. The method as defined in claim 18 wherein the zirconium ion concentration in the rinse solution is about 0.00065 to 0.0050% w/w and the phenolic resin concentration is about 0.01 to 0.40% w/w.

23. The method as defined in claim 18 wherein the zirconium ion concentration in the rinse solution is about 0.00065 to 0.0050% w/w and the phenolic resin concentration is about 0.01 to 0.40% w/w, with a pH of about 3.5 to 5.1.

24. The method as defined in claim 18 wherein the zirconium ion concentration in the rinse solution is about 0.00065 to 0.0011% w/w and the phenolic resin concentration is about 0.01 to 0.077% w/w, with a pH of about 4.0 to 5.1.

25. The method as defined in claim 18 wherein the hafnium ion concentration in the rinse solution is about 0.00035 to 0.0050% w/w and the phenolic resin concentration is about 0.01 to 0.40% w/w.

26. The method as defined in claim 18 wherein the hafnium ion concentration in the rinse solution is about 0.00035 to 0.0050% w/w and the phenolic resin concentration is about 0.01 to 0.40% w/w, with a pH of about 3.5 to 5.1.

27. The method as defined in claim 18 wherein the hafnium ion concentration in the rinse solution is about 0.0008 to 0.0010% w/w and the phenolic resin concentration is about 0.01 to 0.077% w/w, with a pH of about 4.0 to 5.1.

28. The method as defined in claim 18 wherein the titanium ion concentration in the rinse solution is about 0.00035 to 0.0016% w/w and the zirconium concentration is about 0.00065 to 0.0011% w/w and the phenolic resin concentration is about 0.01 to 0.077% w/w, with a pH of about 4.0 to 5.1.

29. The method as defined in claim 18 wherein the titanium ion concentration in the rinse solution is about 0.00035 to 0.0016% w/w and the hafnium concentration is about 0.00035 to 0.0050% w/w and the phenolic resin concentration is about 0.01 to 0.077% w/w, with a pH of about 4.0 to 5.1.

30. A rinse solution as defined in claim 18 wherein the hafnium ion concentration in the rinse solution is about 0.00035 to 0.0050% w/w and the zirconium concentration is about 0.00065 to 0.0011% w/w and the phenolic resin concentration is about 0.01 to 0.077% w/w, with a pH of about 4.0 to 5.1.

31. A rinse solution as defined in claim 18 wherein the titanium ion concentration in the rinse solution is about 0.00035 to 0.0016% w/w and the zirconium concentration is about 0.00065 to 0.0011% w/w and the hafnium ion concentration is about 0.00035 to 0.0050% w/w and the phenolic resin concentration is about 0.01 to 0.077% w/w, with a pH of about 4.0 to 5.1.

32. A rinse solution as defined in claim 18 wherein the titanium ion concentration in the rinse solution is about 0.00035 to 0.001% w/w and the phenolic resin concentration is about 0.01 to 0.077% w/w, with a pH of about 4.0 to 5.1, where the solution is applied by means of spraying.

33. A rinse solution as defined in claim 18 wherein the titanium ion concentration in the rinse solution is about 0.00035 to 0.001% w/w and the phenolic resin concentration is about 0.01 to 0.077% w/w, with a pH of about 4.0 to 5.1, where the solution is applied by means of dipping.

34. The method as defined in claim 18 wherein the Group IVA metal ion is from a Group IVA metal ion source selected from the group consisting of hexafluorozirconic acid, hexafluorotitanic acid, hafnium oxide, titanium oxysulfate, titanium tetrafluoride, zirconium sulfate and mixtures thereof.

35. The method as defined in claim 18 wherein the Group IVA metal ion concentration is about 0.00035 to 0.0050% w/w.

36. A rinse solution as defined in claim 1 wherein the phenolic resin is a mixture of substituted phenol compounds, selected from the group consisting of 2-hydroxybenzyl alcohol, 4-hydroxybenzyl alcohol, 2,6-dimethylol phenol, 2,4-dimethylol phenol and 2,4,6-trimethylol phenol.

37. The method as defined in claim 18 wherein the phenolic resin is a mixture of substituted phenol compounds,

selected from the group consisting of 2-hydroxybenzyl alcohol, 4-hydroxybenzyl alcohol, 2,6-dimethylol phenol, 2,4-dimethylol phenol and 2,4,6-trimethylol phenol.